

# United States Patent Office.

HENRY WURTZ, OF NEW YORK, N. Y.

*Letters Patent No. 60,984, dated January 1, 1867.*

## IMPROVED COMPOSITION OF GLUE OR GELATINE AND OTHER MATERIALS, CALLED DUROGEL.

The Schedule referred to in these Letters Patent and making part of the same.

TO ALL WHOM IT MAY CONCERN:

Be it known that I, HENRY WURTZ, of the city and county of New York, and State of New York, have invented or discovered a new and useful compound, which I designate as Durogel, composed of ordinary glue or gelatine and bichromate of potash, or other compound of chromic acid with the glue. This article may be employed in making buttons, handles of knives, glazing lanterns, and the various uses in which ivory, bone, horn, gutta percha, &c., &c., are employed.

To enable others skilled in the art to make and use the durogel, I would in general terms describe the mode or course of procedure in its manufacture. There may be slight changes, which will readily suggest themselves to the mind of an intelligent operator.

A strong solution in boiling water of common glue is made; say two hundred and fifty parts of glue to five parts of bichromate of potash are heated together, (the bichromate being in a concentrated solution.) Little immediate change is noticeable, except the production of an amber-colored solution; but on cooling and gelatinizing, and this fully dried and exposed to the air and light, it is found to have undergone a profound alteration, being converted into a substance like bone, horn, or ivory. If the application of heat is continued for some time, it loses its fluidity to some extent, and becomes ropy and glutinous. Previous to the addition of the bichromate the solution of glue may be colored by the addition to it of pigments, either transparent in their properties, as roseline and aniline for a beautiful red, verdigris for a green, rouge for a red-brown, &c., &c.; or solid and opaque colors, as lamp-black, the ochres, &c., may be employed. A little acetate of lead gives a fine opaque yellow mass. Fine sand, pounded glass, barytes, may be also used for giving heaviness and hardness to the durogel. Variegated masses may be created by mixing layers of the thinner sheets in different colors, or lumps of different colors may be cemented together. Of course caution must be observed in mixing colors, that none be employed that in their chemical character would affect the bichromate of potash. When the durogel is in thin sheets any liability to over brittleness may be obviated by rubbing the surface with glycerine, which after a time is absorbed by the mass. To build up thick masses it is best to layer the sheets and subject the mass to pressure.

The uses in which this article may be employed are so various that to be particular would be tedious; I would advert to its general employment as a substitute for ivory, bone, gutta percha, vulcanite, in the formation of buttons, glazing lanterns, handles of knives, or other articles of commerce.

Having described in general terms the nature of my improvement, what I claim as my invention, and desire to secure by Letters Patent, is—

The combination of bichromate of potash with ordinary glue or gelatine, in the manner and for the purposes substantially as described in the foregoing specification.

In testimony whereof I have hereunto signed my name before two witnesses.

HENRY WURTZ.

Witnesses:

JOHN F. CLARKE,  
G. WURTZ.